

No. 861,699.

PATENTED JULY 30, 1907

H. G. BARNHURST & J. W. FULLER, JR.  
MODE OF PRODUCING CEMENT CLINKER.

APPLICATION FILED JAN. 22, 1907.



# UNITED STATES PATENT OFFICE.

HENRY G. BARNHURST AND JAMES W. FULLER, JR., OF CATASAUQUA, PENNSYLVANIA.

## MODE OF PRODUCING CEMENT CLINKER.

No. 861,699.

Specification of Letters Patent.

Patented July 30, 1907.

Application filed January 22, 1907. Serial No. 353,516.

*To all whom it may concern:*

Be it known that we, HENRY G. BARNHURST and JAMES W. FULLER, Jr., both citizens of the United States, and residing at Catasauqua, in the county of 5 Lehigh and State of Pennsylvania, have jointly invented certain new and useful Improvements in the Modes of Producing Cement Clinker in the Manufacture of Cement, of which the following is a specification.

10 Our invention has relation to the mode of producing cement clinker, in which certain economies in the quantity and quality of fuel employed in connection therewith are derived, as hereinlater described; and in such general connection our invention relates more 15 particularly to the maintaining and agitating of finely divided raw cement materials and finely divided fuel, mixed together, prior to introduction into a rotary reverberatory kiln, in a non-cohering condition, up to the point of vitrification, fusing or fluxing together of such 20 materials into clinker, with the aid of the said fuel but with such fuel consumed by the time the clinkering is effected.

The principal object of our invention is to provide a mode of producing cement clinker by subjecting finely 25 divided raw cement materials mixed with finely divided fuel, in a rotary reverberatory kiln, to expose grains or particles of the materials and fuel, both in a non-cohering condition to the influence of the highly heated gases and air of the kiln derived from the primary fuel of the kiln as well as to the influence of the highly heated wall of the kiln, the heating of which emanated from the same source, to thereby effect not only a thorough clinkering of the cement materials, but also to obtain a higher resultant efficiency from the 30 combustion of the finely divided fuel mixed with such raw cement materials in the production of the cement clinker, with thereby a great saving in the quantity of fuel employed in the production of a given quantity of cement clinker and with a marked increase of the 35 quantity of clinker obtained in a given time, as compared with the time and quantity and character of fuel hitherto required to convert raw cement materials into blocks, pieces or lumps as well as the supply obtained, for subsequently by grinding or pulverizing bringing 40 45 into the condition of cement, for use.

The nature and scope of our invention will be more fully understood from the following description taken in connection with the accompanying drawings forming part hereof, in which

50 Figure 1, is a view illustrating partly in elevation and partly in section a rotary reverberatory kiln lined with fire-brick, a bin for containing the finely divided dry raw materials and finely divided fuel, means for conducting the mixture of the said materials and of the 55 fuel, both in non-cohering conditions into the rotary reverberatory kiln, and with an outlet for the clinkered

cement material arranged in the wall at the discharge end of the said kiln, the same covering one means, which has been found practically efficient, for carrying into effect the mode of our said invention; and Fig. 2, 60 is a detail view, illustrating in elevation the wall and with an inlet arranged therein for introducing a fuel or the heat of such fuel into the kiln, under the influence of an air blast or suitable feeding device.

Referring to the drawings 3, is a rotary reverberatory 65 kiln, consisting of a metal shell lined with fire brick, which is held in a slightly inclined position from the horizontal and terminates at the lower or discharge end 12, in a wall 6. Preferably in front of the stack 5, and base 4, and in alignment with the kiln 3, is arranged a 70 bin 7, which by means of a conveyer 8, and feeding tube 11, passing partly through the base 4, and stack 5, is connected directly with the kiln. In the bin 7, are placed the raw cement materials to be clinkered, in a dry condition and in a finely divided state, such as 75 cement rock or an equivalent material, as clay, having the same constituents in silica, lime and alumina, as the cement rock and limestone and also the finely divided fuel, consisting of coke or bituminous or anthracite coal, in a dry state, which latter is thoroughly 80 mixed with the raw materials prior to the introduction of both into the kiln 3. The mixture of raw cement materials and fuel in such finely divided and non-cohering state by the conveyer 8, is conducted from the bin 7, into the feeding end 14, of the rotary reverberatory kiln 3, in which the same is advanced by the rotations or movements of such kiln, during treatment 85 therein.

In the wall 6, is arranged an opening 9, through which a fuel such as pulverized coal or the heat of such 90 fuel under the influence of an air blast or feeding device can be introduced into the kiln.

The fuel is introduced at the feeding end 14, of the kiln 3, as well as at the discharge end 12; thereof. The fuel entering at the feeding end 14, is finely pulverized 95 and mixed thoroughly with the finely pulverized cement materials. The fuel introduced at the discharge end 12, of the kiln 3, is termed the primary fuel and that mixed with the cement materials and admitted at the feeding end 14, is termed the secondary fuel and 100 so designated to elucidate the further descriptions of our invention. The kiln is now set in rotation. The flame derived from the primary fuel is permitted to heat up the kiln, the waste heat passing through the chimney 5. The kiln being cylindrical in form and being continuously rotated, while in use, any given transverse section 105 will be equally heated in its whole circumference. When the kiln is highly heated say to a temperature of 2400° Fahrenheit, the charge of raw cement materials with which the secondary fuel is thoroughly mixed is 110 fed in a continuous stream into the feeding end 14, of the kiln 3, by the spout 11, and feed-screw 8, from the

hopper 7. The fuel so mixed with the charge may be bituminous or semi-bituminous coal, coke or anthracite coal, the ash or residue of which being similar in constituents is not detrimental to the qualities of the cement materials being burned. The charge falls from the spout 11, upon adjacent fire brick lining of the kiln 3, and is at once carried away by the rotation of the kiln, the inclined position of which causes the cement materials and secondary fuel to progress and cascade 10 spirally toward the lower or discharge end 12, of the kiln 3. From the heated lining upon which it falls and the flames and gases from the primary fuel playing or reverberating over the same, the charge is caused to be rapidly heated. The kiln being cylindrical and the 15 charge occupying but a small portion of the lower part of the kiln 3, that is, the portion of the lining of the kiln above the charge, is constantly absorbing the heat from the primary fuel. As the fire-bricks thus heated pass under the cascading charge, they impart to the 20 charge a large proportion of the heat thus absorbed. The charge being a fine, non-cohering and non-adhesive powder falls back from the wall of the kiln 3, in cascading exposing every grain or particle of the combined materials to the absorptive influence of heat 25 from the wall and hot products of combustion. As the charge rises in temperature, the fuel entrained therein approaches the point of combustion. As in the case of all burning fuels, the more volatile gases are first disengaged by the increasing heat, and burning add their heat to that of the heat derived from the primary fuel imparting its effect upon the later admitted fuel portions of the charge. As the gases pass off, the fixed carbon is brought to the point of ignition by the heat from the primary fuel. This fixed carbon burns freely absorbing oxygen from the excess air entering the kiln 3, and with the gases and flames of the primary fuel from the discharge end 12. This combustion occurring in 30 contact with the cement materials being treated, the accretion of heat is largely absorbed by the cement materials, which is by it, quickly decarbonized and brought to the point of vitrification. The kiln is given such a rate of rotation as will bring the charge to the point of discharge 10, as fast as vitrification is complete. It is evident that the free access of the heated oxygen 35 of the air to each grain or particle of fuel, as it is exposed in the cascades formed on the continuously rising side of the kiln 3, insures a perfect and uniform combustion of all secondary fuel urged thereto by the heated conditions coming from the primary fuel, augmented 40 by the products of combustion of the secondary fuel in previous charges; the operation being continuous, and the effect cumulative.

The ordinary mode of burning cement materials by the use of the primary fuel only (omitting the pulverized fuel entrained in the charge of cement materials), 45 obtains its efficiency by the direct absorption of its heat passing over the cascading charge and by the indirect transmission of heat taken up by the revolving wall of fire brick, as it passes under the charge. The great rise 50 in the efficiency of the combustion of fuel entrained in the charge as described, permits a decided reduction in the quantity of primary fuel used, the amount of the reduction is very much greater than that required to be mixed with the charge as secondary fuel, this difference 55 represents a large percentage, which is saved as

to the total fuel required to produce the resultant product. The output of the kiln 3, is greatly increased and a much larger quantity of product obtained, owing to the more rapid heating and the more thorough vitrification of the charge in a given time. 70

The conditions for combustion of the secondary fuel mixed with the charges are so perfect that lower grades of coal thus can be made use of, than would be possible under conditions as heretofore existing. The presentation of the secondary fuel and charges under 75 such condition as described, enable the operations to be continuously and uniformly carried on and the fuel to be completely consumed. This must not be confounded with processes, whereby the fuel pulverized or otherwise is permitted to become embedded in 80 masses of coherent cement materials, in which perfect combustion cannot reasonably be expected, and wherein inevitably, much of the fuel must remain as coke or unburned fuel, to the detriment of the product and with the loss of the heat which such unburned portions 85 should have contributed to the operation.

Having thus described the nature and objects of our invention; what we claim as new and desire to secure by Letters Patent is:—

1. The mode of producing cement clinker, which consists 90 in feeding the different raw cement materials thoroughly mixed in separate and non-cohering conditions into one end of a rotary kiln and feeding into the kiln at both ends fuel to be consumed by traveling in opposite directions, the fuel entering the kiln with the raw cement materials by 95 exposing gradually the particles or grains thereof, through the rotary movements of the kiln, producing by the consumption of such in direct contact with the raw materials a complete clinkering of said materials aided in such action by the consumption of the separately introduced fuel. 100

2. The mode of producing cement clinker, which consists 105 in feeding the different raw cement materials thoroughly mixed in separate and non-cohering conditions into one end of a rotary kiln and feeding into both ends fuel, the fuel entering the kiln separately by its consumption highly heating air passing therethrough and the internal walls of the kiln, and the fuel entering the kiln with the different raw cement materials by being exposed to the heated air and walls of the kiln, through rotation of the same and resultant agitation of the raw cement materials therein, 110 causing by its gradual consumption in direct contact with the cement materials the necessary additional heat to effect complete clinkering of said cement materials.

3. The mode of producing cement clinker, which consists 115 in feeding the different raw cement materials thoroughly mixed in separate and non-cohering conditions into one end of a rotary kiln, and feeding into both ends fuel in unequal proportions, the fuel of larger proportion entering the kiln separately by its consumption highly heating the internal walls of the kiln and air passing therethrough, 120 and the fuel of lesser proportion entering the kiln with the raw cement materials by being exposed to the heated air and walls of the kiln through rotation of the same and resultant agitations of the raw cement materials therein, causing by its gradual consumption in direct contact with the cement materials the necessary additional heat to effect complete clinkering of said cement materials. 125

4. The mode of producing cement clinker, which consists 130 in feeding fuels into both ends of a rotary reverberatory kiln; but with one of the fuels, the secondary, in a finely divided state mixed with the raw cement materials in a similar state into an atmosphere, resulting from the hot products of the other fuel, the primary, and admitted air to the kiln, to effect thereby a complete clinkering of the cement materials and the conserving of the ash of the consumed fuel by the combining of the same with the clinkered resultant product. 135

5. The mode of producing cement clinker, which consists 140 in finely dividing the different raw cement materials thor-

oughly mixed and feeding the same in their non-cohering conditions into a rotary kiln and feeding fuel into the kiln therewith to conjointly act by its consumption upon all separated non-cohering particles of said materials to effect 5 thereby a quick and thorough clinkering thereof.

6. The mode of producing cement clinker, which consists in introducing fuel at different points into a rotary kiln, the fuel from one point to fire and maintain the kiln in a highly heated condition and the fuel from the other mixed 10 with the different raw cement materials in non-cohering conditions to effect by its combustion the perfect or com-

plete clinkering of the grains or particles of the different cement materials aided by the products of the separately introduced fuel of the kiln.

In witness whereof, we have hereunto affixed our signatures in the presence of the two subscribing witnesses. 15

HENRY G. BARNHURST.  
JAMES W. FULLER, JR.

Witnesses:

J. WALTER DOUGLASS,  
GEO. W. REED.